

# United States Patent

[19]

Takechi et al.

[11] 3,925,111

[45] Dec. 9, 1975

[54] **HIGH TENSILE STRENGTH AND STEEL  
AND METHOD FOR MANUFACTURING  
SAME**

[75] Inventors: **Hiroshi Takechi; Tsuyoshi Kawano,**  
both of Kisarazu; **Toshio  
Hashizume; Kazuo Koyama,** both of  
Kimitsu; **Hiroaki Masui,** Chiba, all  
of Japan

[73] Assignee: **Nippon Steel Corporation,** Tokyo,  
Japan

[22] Filed: **Dec. 28, 1973**

[21] Appl. No.: **429,274**

[30] **Foreign Application Priority Data**

Dec. 31, 1972 Japan..... 48-2832  
Dec. 31, 1972 Japan..... 48-2833

[52] **U.S. Cl.**..... 148/12 F

[51] **Int. Cl.<sup>2</sup>**..... C21D 7/14

[58] **Field of Search**..... 148/12 F, 12 C

[56] **References Cited**

UNITED STATES PATENTS

|           |         |                    |          |
|-----------|---------|--------------------|----------|
| 3,328,211 | 6/1967  | Nakamura .....     | 148/12 F |
| 3,432,368 | 3/1969  | Nakamura .....     | 148/12 F |
| 3,544,393 | 12/1970 | Zanetti .....      | 148/12 F |
| 3,625,780 | 12/1971 | Bosch et al. ....  | 148/12 F |
| 3,673,007 | 6/1972  | Miyano et al. .... | 148/12 F |

*Primary Examiner*—W. Stallard

*Attorney, Agent, or Firm*—Toren, McGeady and  
Stanger

[57] **ABSTRACT**

Method of manufacturing of high tensile steel having superior cold workability and excellent toughness characterized in that when Ti added Al killed steel, which contains 0.04 to 0.35% of Ti, under the condition of  $Ti/C < 4$ , and 0.005, to 0.15% of sol Al, is finishing its hot rolling in a temperature range of 815° to 880°C, at least more than one time of large reduction of more than 28% of draft percentage for one pass are given in a temperature range of 980° to 1100°C.

**9 Claims, No Drawings**

## HIGH TENSILE STRENGTH AND STEEL AND METHOD FOR MANUFACTURING SAME

### DETAILED EXPLANATION OF THE INVENTION

This invention relates to a method for manufacturing high tensile steel, having more than 60 Kg/mm<sup>2</sup> of tensile strength as rolled and at the same time having superior cold workability and excellent low temperature toughness, preferably from a hot rolled steel plate having more than 4.5 mm of thickness.

Important characteristics required for high tensile steel having more than 60 Kg/mm<sup>2</sup> grade, tensile strength toughness, weldability, cold workability and the like are, and the usual high tensile steel plate may be classified into two types. One type is where the toughness and weldability are regarded as important, since they are mainly used for shipbuilding steel and structural steel. In this case, a thermal refined steel is used which is relatively thick and is mainly subjected to quenching and tempering and the like. Its most important characteristics are toughness and weldability, and it possesses little cold workability properties. The other type is steel plate having a comparatively small thickness (for instance, less than 9 mm) which is used for truck frames and the like. In case, its most important characteristic is superior cold workability which is bearable under severe cold working, and particularly under bending working and hole expanding working, while toughness and the like are not as important.

But, recently high tensile steel having a strength of 60-80 Kg/mm<sup>2</sup> grade has come to be used even for steel plate for cold working.

In general, the cold workability, toughness and weldability of steel will decrease as its strength increases, so that even high tensile steel for cold working cannot ignore the low temperature toughness of a portion of the plastic deformation in deference to the cold workability. Thus, high tensile steel having inferior low temperature toughness is in danger of brittle fracture during its use, particularly in cold districts, even though its cold workability is excellent. Therefore, in high tensile steel having a thickness of more than 4.5 mm, it is required to have superior low temperature toughness in addition to cold workability.

Because of this, attempts to develop a high tensile steel, which is superior, not only in cold workability, but also in low temperature toughness and weldability. However, the high tensile steel that satisfied all of these required characteristics was very limited and expensive.

Usually, as a high tensile steel for cold working, niobium added steel and vanadium added steel have been widely used. These steel are superior in toughness, however, they have such disadvantages that the strength of niobium steel is limited up to 60 Kg/mm<sup>2</sup> grade and vanadium steel may be produced up to 70 Kg/mm<sup>2</sup> grade but is expensive.

Recently, instead of niobium or vanadium steel, titanium added high tensile steel has been investigated. The titanium added steel has the advantage of being cheaper than niobium steel or vanadium steel and is superior in cold workability. But on the other hand, it is inferior to such steels in toughness which is an essential characteristics of a high tensile steel of more than 4.5 mm of thickness.

The inventors have succeeded in manufacturing high tensile steel plate having a strength of more than 60 Kg/mm<sup>2</sup> as rolled, and at the same time, superior toughness and weldability in addition to superior cold workability, by means of manufacturing a titanium added steel having an appropriate composition range under specified hot rolling conditions.

The essential points of the method according to the invention may be enumerated as follows.

- 10 1. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 815° to 880°C, at least more than one time of large reduction of more than 28% of draft percentage for one pass are given in a temperature range of 980° to 1100°C.
  - 15 2. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 730° to 815°C, total draft percentage below 980°C is made more than 50%.
  - 20 3. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 730° to 815°C, total draft percentage below 980°C is made more than 50%.
  - 25 4. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 730° to 815°C, total draft percentage below 980°C is made more than 50%.
  - 30 5. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 730° to 815°C, total draft percentage below 980°C is made more than 50%.
  - 35 6. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 730° to 815°C, total draft percentage below 980°C is made more than 50%.
  - 40 7. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 730° to 815°C, total draft percentage below 980°C is made more than 50%.
  - 45 8. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 730° to 815°C, total draft percentage below 980°C is made more than 50%.
  - 50 9. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 730° to 815°C, total draft percentage below 980°C is made more than 50%.
  - 55 10. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 730° to 815°C, total draft percentage below 980°C is made more than 50%.
  - 60 11. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 730° to 815°C, total draft percentage below 980°C is made more than 50%.
  - 65 12. Method for manufacturing of high tensile steel having superior cold workability and excellent toughness characterized in that when Ti added Al killed steel, which contains 0.04 to 0.35% of Ti, under the condition of Ti/C<4, and 0.005 to 0.15% of Sol Al, is finishing its hot rolling in a temperature range of 730° to 815°C, total draft percentage below 980°C is made more than 50%.
- In the invention, the reasons for limitation of preferred chemical compositions and rolling conditions are described as follows:

C is necessary for obtaining a strength of more than 60 Kg/mm<sup>2</sup> and this object cannot be attained with less than 0.03% C, while more than 0.20% C will result in inferior cold workability, low temperature toughness and weldability. The preferable range for the carbon is 0.05 to 0.15% C.

Ti is a very important element for the invention, because it will remarkably increase the strength of the steel by the precipitation of fine Ti(CN), Ti(CN), and at the same time decrease the plasticity of the non-metallic inclusion and increase the cold workability and impact absorbed energy in the transverse direction. But, the object of the invention cannot be attained by less than 0.04% Ti, while its effect will be saturated with more than 0.35% Ti. It is preferable to add 0.05 to 0.30% Ti in order to realize the characteristics of the invention. Also, it is necessary to make Ti/C<4 to increase the strength efficiently, and when the ratio becomes more than 4, the strength of the steel will decrease.

Si is effective to increase the strength, but when it becomes more than 0.8%, the toughness and weldability will become inferior, so that its upper limit is made as 0.8%. However, if Si is not necessary for the strength, it may not be added. However, normally it is preferable to add more than 0.10% Si in order to obtain the desired strength.

Mn is an essential element to make the steel strong and tough. In the invention, less than 0.9% Mn is effective, and the cold workability is decreased with more than 2.5% Mn, so that the upper limit is 2.5%, but it is preferable to add less than 2.0% Mn in order to minimize the appearance of the upper bainite structure, which is harmful to the toughness.

Al is necessary with 0.005 to 0.15% thereof being present as acid soluble Al to assure the effectiveness of to Ti.

The preferable range is 0.01 to 0.10% sol Al.

S and N are deleterious elements in the steel of the invention, because they will combine with Ti and decrease the amount of effective Ti which will act on the reinforcement of the steel.

Reduction of S and N is extremely effective to toughen the steel, and it is necessary to make the S less than 0.020% and the N less than 0.0080%, respectively, to stabilize the characteristics of the invention.

Advantageously, it is preferred that S and N contents are as small as possible, i.e., S is less than 0.010% and N is less than 0.0060%. Additionally, one or more of the undermentioned elements may be added as occasion demands for the purposes indicated.

Zr will fix the N and S in the steel to increase the effectiveness of the Ti and to improve the characteristics of the invention, so that it is a very important element. However, less than 0.01% Zr is not effective and its effect will be saturated with more than 0.15% Zr. The optimum content of Zr is 0.03 to 0.06%.

Mischmetal will also fix the S in the steel and improve the effectiveness of the Ti as well as the cold workability and toughness. When the mischmetal is present, no effect is observed if (La + Ce) is less than 0.005%, and the effect is saturated if (La + Ce) is more than 0.10%. The optimum content thereof is (La + Ce) = 0.005-0.05%.

Nb and V will toughen steel by way of grain refining and stabilize the effect of the invention, and also V will fix N which is deleterious to the invention, so that both of these are effective elements in the steel of the invention.

tion. But neither has any effect in the range of less than 0.01%, and in the range of more than 0.10%, not only is the effect is, but the steel becomes very expensive. The optimum content thereof is 0.01 to 0.05%, respectively.

Ni, Cr and Cu will lower the transformation temperature (Ar<sub>3</sub>) of steel and are effective for toughening the steel as well as improving the corrosion resistance thereof, so that less than 0.5% of each may be added if needed.

B will fix N which is deleterious to the invention and increase the strength of steel, so that less than 0.0030% thereof may be added if needed.

The reasons for limiting the rolling conditions are as follows.

In the first place, as to the heating temperature for the slab, in order to obtain high strength, it is necessary to elevate the heating temperature so as to maximize the solid solution of Ti in the austenite structure, and to assure a tensile strength of more than 60 Kg/mm<sup>2</sup>, which being the object of the invention. Particularly, it is necessary to make the heating temperature more than 1200°C, and, it is preferable to make the temperature more than 1260°C for 70 Kg/mm<sup>2</sup> grade and more than 1280°C for 80 Kg/mm<sup>2</sup> grade.

In the next place, the rolling conditions are particularly important in the invention. Namely, the heating temperature for slab is made high to obtain the highest strength in the invention, but under the condition of ordinary hot rolling, the low temperature toughness of steel is remarkably lowered. This is because the austenite grains become remarkably coarse, and in titanium contained steel as well as niobium steel, the low temperature toughness will decrease if the heating temperature is raised to improve the strength. Conversely, if low temperature heating is effected to improve the low temperature toughness, the strength of steel will be lowered. Moreover, the titanium containing steel shows a more remarkable deterioration in toughness from high temperature heating compared with the niobium containing steel.

The inventors succeeded in developing of high tensile steel plate which has high strength, superior toughness and cold workability at the same time by specifying the rolling condition, as the result of various researches about methods for improving toughness for titanium containing steel which is heated at a temperature of more than 1200°C.

In the invention, the object is attained by two kinds of rolling conditions, i.e., the high temperature finishing type and low temperature finishing type.

In the first place, the rolling condition of the high temperature finishing type will be explained. Namely, as the result of detailed research of rolling conditions of titanium containing steel within the composition range of the invention, it was found that even in Ti added steel, austenite grains which became coarse by heating will surely recrystallize into new fine grains by rolling at a temperature of more than 1100°C. Also, we have found that if in rolling at less than 1100°C a large reduction of more than 28% of draft percentage for one pass is effected, recrystallization become possible down to 980°C and the grains also become smaller. Moreover, even if the finishing temperature is as high as 880°C, at which temperature the rolling will normally be completed, cold workability and low temperature toughness are remarkably improved. As the result of various further researches, we found that, in hot rolling

process after heating of heating slab, by effecting a with more than one pass and with a draft percentage for one pass of more than 28% between 1100°-980° C, and making the finishing temperature of rolling lower than 880°C and higher than 730°C, titanium containing high tensile steel plate is obtained, which has superior cold workability and remarkably improved low temperature toughness. Thus, these are the specified rolling conditions of the high temperature finishing type in the present invention.

The characteristic of this high temperature finishing type resides in that said specific rolling of large reduction is effected more than one time between 1100°-980°C, and of course the more times of said large reduction are effected, the more preferable. In this case, the rolling conditions over 1100°C are not specified, because when the rolling at higher than 1100°C is effected according to the conventional schedule (normally a total draft percentage of more than 50%) and in succession said specific large reduction is effected between 1100°-980°C, the structure will recrystallize into finer austenite grains. Further, when the decrease of productivity is not a problem, steel having very superior cold workability and low temperature toughness can be obtained by omitting entirely the rolling at higher than 1100°C and by effecting a number of specific large reductions between 1100°-980°C.

In this high temperature finishing type, further rolling is effected after the specific large reduction rolling, and the rolling is finished below 880°C and over 730°C to give higher toughness and higher cold workability. This is done so that the recrystallized austenite grains are further rolled within a temperature range wherein recrystallization of austenite is impossible to make the ferrite grains fine after transformation, and thereby the low temperature toughness, particularly at the transition temperature, is improved as well as the superior cold workability are improved. Moreover, we recommend that total reduction below 980° C be more than 45% (preferably 50%) to realize the characteristics of the invention.

The reasons for limiting the rolling condition of high temperature finishing type are as above mentioned. However, said specific large reduction between 1100°-980° C is not always possible in all rolling mills. In such rolling mills, the object of the invention may be attained by means of the low temperature finishing method.

In the low temperature finishing type of the invention, the rolling condition in the low temperature region is particularly important. Namely, since the finely recrystallized austenite grains cannot be obtained as in the high temperature finishing type, the structure after transformation is liable to become a ferrite structure of mixed grains or mixed with an upper bainite structure, and steel having such a structure is remarkably inferior in low temperature toughness and cold workability. To solve such a problem, it is necessary to effect a larger reduction in a lower temperature region than the high temperature finishing type in order to make the ferrite grains, after transformation, fine and uniform. As the result of various experiments, it has been clarified that the cold workability and the low temperature toughness are remarkably improved by making the total draft percentage below 980°C more than 50% and by finishing the rolling at a temperature lower than 815°C and higher than 730°C, and this is the specified rolling con-

ditions of the low temperature finishing method in the present invention. In addition, by making the total draft percentage below 850°C more than 20%, the cold workability and the low temperature toughness can be improved further. The rolling conditions at higher than 980°C are not specified, because the object of the invention can be attained so long as the rolling schedule at above 980°C which has been effected conventionally (normally the total draft percentage at higher than 980°C is effected with more than 60%) is performed and the rolling conditions in the low temperature region are satisfied according to the invention.

When the decrease of productivity is not a problem, the characteristics of the invention may be improved by minimizing the rolling at higher than 1100°C and by increasing the total draft percentage below 1100°C. However, this is not a preferred method, because the productivity will be remarkably decreased and improvement of the quality of steel is not great.

The difference between the two types of rolling described above is that the former is available for higher rolling finishing temperatures and, therefore has high productivity and, as shown in some examples, the higher the rolling finishing temperature the higher strength can be obtained, so that it the high temperature finishing type is preferred.

But, in rolling mills which cannot carry out the high temperature finishing type, the object of the invention can be attained by adopting the low temperature finishing type, even though the strength will somewhat decrease.

Even in the high temperature finishing type, by finishing the rolling below 815° and above 730°C, which is the rolling finishing temperature of the low temperature finishing type, the low temperature toughness, particularly the transition temperature, is improved much more and has a superior transition temperature than the low temperature finishing type, so that in the invention, even in the high temperature finishing type, the rolling finishing temperature is below 880° and above 730°C.

After the rolling is finished the steel may be air-cooled in plate shape as is carried out in the ordinary thick plate process, or taken up in the coil shape. However, higher strength may be obtained when water-cooled and coiled. In case the steel is coiled, the characteristics of the invention may be displayed to the utmost, by making the coiling temperature 500° to 680°C and by making the cooling velocity from the finish of rolling to the coiling (hereinafter simply called the cooling velocity) between 3° and 40°C/sec.

The invention will be further explained by the following examples.

#### Example 1.

##### (High temperature finishing type)

Table 2 shows various values of the characteristics of hot rolled steel plate having thickness of 8mm, which is obtained by rolling of the steel shown in Table 1 subject to the rolling condition shown in Table 2, i.e. mechanical properties of the hot rolled steel plate; minimum radius capable of bending 180° in the transverse direction (width of test piece = 200mm) and hole expanding limit (initial hole diameter = 20mm); vE-20 after 5% tensile strain representing low temperature toughness after cold working and vE-20 without pre-strain.

As is clear from Table 2, it is apparent that according to the high temperature finishing type (No. of rolling 2-5, 8-14) of the method of the invention, cold workability and low temperature toughness of steel plate are remarkably improved compared with the comparative method (No. of rolling 1, 6, 7, 15).

#### EXAMPLE 2

##### (High Temperature Finishing Type)

Chemical compositions of the steel according to the invention and the comparative steel are shown in Table 3. These steels are molten and produced in converters, and after they are formed as slabs by way of ordinary process, they are rolled subject to the rolling condition shown in Table 4 into hot rolled steel plates of 8.0 mm thickness, of which various values of characteristics are shown in Table 4. And, coiling temperatures were 580°-620°C, and cooling velocity 7°-11°C/sec.

Even in the case of steel having chemical compositions within the range of the invention, products having rolling numbers 16 and 19, which do not satisfy the rolling condition of the invention, are of the same grade in cold workability compared with rolled products from the comparative steel (No. of rolling 22,23), but low temperature toughness are inferior.

The rolled products having rolling numbers 17, 18, 20 and 21 according to the high temperature finishing type of the invention have higher strength than the rolled products from the comparative steel. Moreover cold workability of the invention steels is remarkably more superior than those from the comparative steel and also their low temperature toughness is more than or equal to those from the comparative steel plate.

#### EXAMPLE 3

##### (High Temperature Finishing Type)

Chemical compositions of the steel according to the invention and the comparative steel are shown in Table 5. These steels are molten and produced in converters, and after they are formed as slabs by way of ordinary process, they are rolled subject to the rolling condition shown in Table 6 into hot rolled steel plates of 6.0-10.0mm thickness, of which various values of characteristics are shown in Table 7.

As is clear from Table 7, the hot rolled steel plates produced according to the high temperature finishing type of the invention have higher strength and superior cold workability to any comparative steel as well as superior low temperature toughness more than or equal to the comparative steel.

Steel 2 of the invention made by adding Zr to steel 1 of the invention and steel 3 of the invention made by adding Nb and V to steel 1 are more improved than steel 1 of the invention in any of strength, cold workability and low temperature toughness, thus it is understood that the effect of the invention is still more displayed by the addition of Zr, Nb and V.

#### EXAMPLE 4

##### (Low Temperature Finishing Type)

Table 8 shows various values of the characteristics of hot rolled steel plate having thickness of 8mm, which is obtained by rolling of the steel shown in Table 1 subject to the rolling condition shown in Table 8, i.e. mechanical properties of the hot rolled steel plate; minimum radius capable of bending 180° in the transverse direction

and hole expanding limit representing cold workability of high tensile steel plate; and vE-20 after 5% tensile strain representing low temperature toughness after cold working and vE-20 without pre-strain.

As is clear from Table 8, according to the low temperature finishing type (No. of rolling 28, 29, 32, 33, 34) of the invention, the cold workability and the low temperature of the steel plate are remarkably improved compared with the comparative method (No. of rolling 25, 26, 27, 30, 31, 35, 36).

#### EXAMPLE 5

##### (Low Temperature Finishing Type)

Steel according to the invention and comparative steel having chemical compositions shown in Table 3 are rolled subject to the rolling condition shown in Table 9 into hot rolled steel plate of 8.0mm thickness, of which various kinds of characteristic values are shown in Table 9. And, coiling temperature therefor are 580°-620°C and cooling velocity from the end of rolling to the coiling are 7°-11°C/sec.

Even though steel having chemical compositions within the range of the invention is used, the steel plate having rolling number 37, which does not satisfy the rolling condition of the invention, has equal cold workability to comparative steel plate (rolling number 22, 23), but the low temperature is inferior to the comparative steel plate.

The steel plate having rolling number 38 obtained according to the low temperature finishing type of the method of the invention has higher strength than comparative steel, nevertheless cold workability of the invention steel plate is remarkably superior and low temperature toughness thereof has characteristics of more than or equal to comparative steel plate.

#### EXAMPLE 6

##### (Low Temperature Finishing Type)

Chemical compositions of the steel within the range of the invention and of the comparative steel are shown in Table 5. These steels are rolled subject to rolling condition shown in Table 10 into hot rolled steel plate having thickness of 6.0-10.0mm, of which various kinds of characteristic values are shown in Table 11. As is clear from Table 11, the hot rolled steel plate formed according to the low temperature finishing type of the invention has higher strength and superior cold workability to the comparative steel as well as superior low temperature toughness more than or equal to the comparative steel. Steel 2 of the invention made by adding Zr to steel 1 of the invention and steel 3 of the invention made by adding Nb and V to steel 1 are more improved than steel 1 of the invention in any of strength, cold workability and low temperature toughness, thus it is understood that the effect of the invention is still more displayed by the addition of Zr, Nb and V.

Having thus described the invention in details, the high tensile steel plate produced according to the invention has strength of more than 60 Kg/mm<sup>2</sup>, having superior cold workability and low temperature toughness at the same time compared with usual high strength steel plates, and its carbon equivalent is low so that its weldability is very good. Among cold workabilities, drawability and stretchability are more than or equal to those of usual steel, so that the high tensile steel of the invention is not only adapted for automobile frame and the like but also best suited for making

line-pipe because of good low temperature toughness and good weldability. Particularly, the present steel as  $V_{-40}^E$  2.1 kg-m and  $V_{rs}^T$  60°C according to JIS No. 4, 5mm sub size specimen.

Table 1

| C    | Si   | Mn   | Chemical Compositions of Examples 1 and 4 (wt%) |       |      |         |        |     | Ti/C                       | Rest |
|------|------|------|-------------------------------------------------|-------|------|---------|--------|-----|----------------------------|------|
|      |      |      | P                                               | S     | Ti   | Sol. Al | N      |     |                            |      |
| 0.10 | 0.33 | 1.27 | 0.012                                           | 0.006 | 0.12 | 0.031   | 0.0040 | 1.2 | Fe and inevitable elements |      |

Table 2

| Rolling conditions and various kinds of characteristic values of Example 1 |             |                            |                                         |                                          |                                        |                                          |                              |                              |  |  |  |  |
|----------------------------------------------------------------------------|-------------|----------------------------|-----------------------------------------|------------------------------------------|----------------------------------------|------------------------------------------|------------------------------|------------------------------|--|--|--|--|
| Rolling pattern                                                            | Rolling No. | Heating temp. of slab (°C) | Rolling Condition                       |                                          | Total draft percentage below 980°C (%) | Total draft percentage above 1100°C (%)  | Rolling between 1100°C/980°C | Rolling finishing temp. (°C) |  |  |  |  |
|                                                                            |             |                            | Total draft percentage above 1100°C (%) | Rolling between 1100°C/980°C             |                                        |                                          |                              |                              |  |  |  |  |
| C                                                                          | 1           | 1300°C                     | 53%                                     | → 29% → 51.5%<br>(Times of pass=1)       | 51.5%                                  | → 31% → 34% → 51.5%<br>(Times of pass=2) | 840                          | 920                          |  |  |  |  |
|                                                                            | 2           |                            |                                         |                                          |                                        |                                          |                              | 880                          |  |  |  |  |
|                                                                            | 3           |                            |                                         |                                          |                                        |                                          |                              | 840                          |  |  |  |  |
|                                                                            | 4           |                            |                                         |                                          |                                        |                                          |                              | 800                          |  |  |  |  |
|                                                                            | 5           |                            |                                         |                                          |                                        |                                          |                              | 750                          |  |  |  |  |
|                                                                            | 6           |                            |                                         |                                          |                                        |                                          |                              | 710                          |  |  |  |  |
| D                                                                          | 7           | 1300°C                     | 28%                                     | → 31% → 34% → 51.5%<br>(Times of pass=2) | 51.5%                                  | → 30% → 48.0%<br>(Times of pass=1)       | 840                          | 920                          |  |  |  |  |
|                                                                            | 8           |                            |                                         |                                          |                                        |                                          |                              | 880                          |  |  |  |  |
|                                                                            | 9           |                            |                                         |                                          |                                        |                                          |                              | 840                          |  |  |  |  |
| E                                                                          | 10          | 1300°C                     | 49%                                     | → 30% → 48.0%<br>(Times of pass=1)       | 48.0%                                  | → 25% → 52.4%<br>(Times of pass=1)       | 840                          | 880                          |  |  |  |  |
|                                                                            | 11          |                            |                                         |                                          |                                        |                                          |                              | 840                          |  |  |  |  |
| F                                                                          | 12          | 1300°C                     | 55%                                     | → 25% → 52.4%<br>(Times of pass=1)       | 52.4%                                  | 840                                      | 860                          | 860                          |  |  |  |  |
|                                                                            | 13          |                            |                                         |                                          |                                        |                                          |                              | 860                          |  |  |  |  |
| F                                                                          | 14          | 1300°C                     | 55%                                     |                                          |                                        |                                          |                              | 860                          |  |  |  |  |
|                                                                            | 15          |                            |                                         |                                          |                                        |                                          |                              | 860                          |  |  |  |  |

## Note.

1) Encircled "Rolling No." are belonging to the invention.

2) Water-cooling is effected from the end of rolling to 600°C with velocity of 10°C/sec, then furnace cooling from 600°C.

| Mechanical Properties<br>(JIS No. 5) | Cold Workability                  |                                        |                |                                                                                           | Low temperature toughness (JIS No. 4, sub-size 7.5mm) |                    |                           |
|--------------------------------------|-----------------------------------|----------------------------------------|----------------|-------------------------------------------------------------------------------------------|-------------------------------------------------------|--------------------|---------------------------|
|                                      | Yield point (Kg/mm <sup>2</sup> ) | Tensile strength (Kg/mm <sup>2</sup> ) | Elongation (%) | Minimum radius capable of 180° bending in transverse direction (test piece width = 200mm) | Hole expanding limit (d/do) (do=20mm)                 | without pre-strain | after 5% tensile strength |
| 65.7                                 | 74.0                              | 27                                     | 0.5 t          | 2.1                                                                                       | 7.8                                                   | 1.5                |                           |
| 66.0                                 | 74.1                              | 28.5                                   | 0 t            | 2.7                                                                                       | 10.6                                                  | 8.0                |                           |
| 62.8                                 | 70.1                              | 29                                     | 0 t            | 2.7                                                                                       | 12.1                                                  | 9.4                |                           |
| 61.3                                 | 68.7                              | 29                                     | 0 t            | 2.9                                                                                       | 13.4                                                  | 11.3               |                           |
| 61.5                                 | 66.8                              | 30                                     | 0 t            | 2.7                                                                                       | 12.1                                                  | 10.4               |                           |
| 60.8                                 | 65.8                              | 30                                     | 0.5 t          | 2.2                                                                                       | 8.7                                                   | 4.6                |                           |
| 64.8                                 | 73.2                              | 26.5                                   | 0.5 t          | 2.2                                                                                       | 6.9                                                   | 1.9                |                           |
| 63.1                                 | 72.1                              | 27                                     | 0 t            | 2.7                                                                                       | 11.3                                                  | 8.8                |                           |
| 63.8                                 | 71.3                              | 28                                     | 0 t            | 2.8                                                                                       | 12.6                                                  | 10.4               |                           |
| 60.9                                 | 67.8                              | 29                                     | 0 t            | 2.8                                                                                       | 13.1                                                  | 11.0               |                           |
| 60.1                                 | 67.5                              | 29                                     | 0 t            | 2.9                                                                                       | 12.8                                                  | 11.4               |                           |
| 64.4                                 | 72.4                              | 28                                     | 0 t            | 2.4                                                                                       | 9.2                                                   | 5.7                |                           |
| 63.1                                 | 70.6                              | 29                                     | 0 t            | 2.5                                                                                       | 9.9                                                   | 7.6                |                           |
| 60.8                                 | 68.4                              | 30                                     | 0 t            | 2.7                                                                                       | 11.0                                                  | 9.8                |                           |
| 64.2                                 | 72.1                              | 27                                     | 0.5 t          | 2.2                                                                                       | 7.3                                                   | 2.0                |                           |

possesses an excellent low temperature toughness such

Table 3

| C                                        | Si   | Mn   | Chemical compositions of Examples 2 and 5 (wt%) |       |         |       |      |        | Ti/C | Nb   | Rest                      |
|------------------------------------------|------|------|-------------------------------------------------|-------|---------|-------|------|--------|------|------|---------------------------|
|                                          |      |      | P                                               | S     | Sol. Al | Ti    | N    |        |      |      |                           |
| Steel of the invention comparative steel | 0.12 | 0.35 | 1.43                                            | 0.017 | 0.006   | 0.034 | 0.09 | 0.0032 | 0.75 | —    | Fe and inevitable element |
|                                          | 0.09 | 0.27 | 1.31                                            | 0.018 | 0.008   | 0.025 | —    | 0.0048 | —    | 0.04 |                           |

Table 4

| Rolling conditions and various kinds of characteristic values of Example 2 |                 |             |                            |                                     |                                            |                                    |                              |  |
|----------------------------------------------------------------------------|-----------------|-------------|----------------------------|-------------------------------------|--------------------------------------------|------------------------------------|------------------------------|--|
| Kind of Steel                                                              | Rolling pattern | Rolling No. | Heating temp. of slab (°C) | Rolling Conditions                  |                                            | Total draft percentage below 980°C | Rolling finishing temp. (°C) |  |
|                                                                            |                 |             |                            | Total draft percentage above 1100°C | Each draft percentage between 1100°C/980°C |                                    |                              |  |
| Steel of the invention                                                     | G               | 16 (7)      | 1270°C                     | 56%                                 | → 30% →<br>→ 35% →<br>(Times of pass=2)    | 73%                                | 900<br>850<br>800            |  |
| Comparative Steel                                                          | H               | 19 (20)     | 1270°C                     | 69%                                 | → 35% →<br>(Times of pass=1)               | 73%                                | 900<br>850<br>800            |  |
|                                                                            | I               | 22          | 1270°C                     | 64%                                 | → 25% →<br>25 →<br>(Times of pass=2)       | 73%                                | 850                          |  |
|                                                                            | H               | 23          | 1270°C                     | 69%                                 | → 35% →<br>Times of pass=1)                | 73%                                | 850                          |  |

## Note:

1) Encircles "Rolling No." are belonging to the invention

2) Coiling temperature = 580° to 620°C

3) Cooling velocity = 7° to 11°C/sec.

| Mechanical Properties (JIS No. 5) |                           |                | Cold Workability                                                                        |                                       |                    | Low temperature toughness(JIS No. 4,sub-size 7.5mm) |                     | Remarks |
|-----------------------------------|---------------------------|----------------|-----------------------------------------------------------------------------------------|---------------------------------------|--------------------|-----------------------------------------------------|---------------------|---------|
| Yield point (Kg/mm²)              | Tensile strength (Kg/mm²) | Elongation (%) | Minimum radius capable of 180° bending in transverse direction test piece (width=200mm) | Hole expanding limit (d/do) (do=20mm) | without pre-strain | after 5% tensile strain                             | vE-20 (Kg-m)        |         |
| 66.1                              | 72.1                      | 26             | 0.5 t                                                                                   | 1.9                                   | 6.4                | 2.0                                                 | Comparative example |         |
| 61.9                              | 68.4                      | 28             | 0 t                                                                                     | 2.8                                   | 11.3               | 10.2                                                |                     |         |
| 59.7                              | 66.8                      | 29             | 0 t                                                                                     | 2.9                                   | 12.1               | 10.5                                                | The invention "     |         |
| 64.2                              | 71.9                      | 27             | 0.5 t                                                                                   | 1.9                                   | 5.8                | 1.9                                                 | Comparative         |         |
| 61.2                              | 68.4                      | 29             | 0 t                                                                                     | 2.7                                   | 10.4               | 8.7                                                 | The invention       |         |
| 59.4                              | 65.4                      | 30             | 0 t                                                                                     | 2.7                                   | 11.8               | 9.8                                                 | "                   |         |
| 50.6                              | 63.4                      | 32             | 0.5 t                                                                                   | 1.9                                   | 9.8                | 7.8                                                 |                     |         |
| 51.7                              | 62.7                      | 33             | 0.5 t                                                                                   | 1.8                                   | 10.6               | 8.5                                                 |                     |         |

Table 5

| Chemical Compositions of Examples 3 and 6 (wt %) |      |      |      |       |       |        |        |      |      |                     |                            |
|--------------------------------------------------|------|------|------|-------|-------|--------|--------|------|------|---------------------|----------------------------|
|                                                  | C    | Si   | Mn   | P     | S     | sol.Al | N      | Ti   | Ti/C | Others              | Rest                       |
| Steel 1 of the invention                         | 0.11 | 0.33 | 1.45 | 0.017 | 0.006 | 0.032  | 0.0044 | 0.18 | 1.64 | 0.04% Zr            |                            |
| Steel 2 "                                        | 0.11 | 0.33 | 1.45 | 0.017 | 0.006 | 0.032  | 0.0044 | 0.18 | 1.64 | 0.02% Nb, 0.01% V   | Fe and inevitable elements |
| Steel 3 "                                        | 0.11 | 0.33 | 1.45 | 0.017 | 0.006 | 0.032  | 0.0044 | 0.18 | 1.64 | 0.02% Nb, 0.01% V   |                            |
| Steel 4 "                                        | 0.10 | 0.37 | 1.48 | 0.018 | 0.005 | 0.035  | 0.0052 | 0.21 | 2.10 | 0.35% Cr, 0.0015% B |                            |
| Steel 5 "                                        | 0.08 | 0.41 | 1.38 | 0.012 | 0.008 | 0.045  | 0.0047 | 0.10 | 1.25 | 0.24% Ni, 0.32% Cu  |                            |
| Steel 6 "                                        | 0.10 | 0.26 | 1.10 | 0.011 | 0.008 | 0.018  | 0.0048 | 0.10 | 1.0  | 0.02% (La+Ce)       |                            |
| Comparative steel                                | 0.09 | 0.27 | 1.27 | 0.013 | 0.007 | 0.028  | 0.0051 | —    | —    | 0.04% Nb, 0.03% V   |                            |

Table 6

| Rolling conditions of Example 3 |                       |                            |                           |                           |                   |               |                  |
|---------------------------------|-----------------------|----------------------------|---------------------------|---------------------------|-------------------|---------------|------------------|
| Rolling pattern                 | Heating temp. of slab | Total draft % above 1100°C | Each draft % between      | Total draft % below 980°C | Rolling finishing | cooling temp. | Cooling velocity |
| High temp. finishing type       | 1260–1320°C           | More than 50%              | →35% →<br>times of pass=1 | more than 50%             | 840°–870°         | 570–620°C     | 3–13°C/sec       |

Table 7

| Various kinds of characteristic values of steel plates obtained by Example 3 |                           |                           |                                   |                                        |                           |                                                                                         |                                       |                         |      |
|------------------------------------------------------------------------------|---------------------------|---------------------------|-----------------------------------|----------------------------------------|---------------------------|-----------------------------------------------------------------------------------------|---------------------------------------|-------------------------|------|
| Manufacturing condition                                                      | Mechanical property       |                           | Cold workability                  |                                        | Low temperature toughness |                                                                                         |                                       |                         |      |
|                                                                              | Rolling pattern           | Thickness of product (mm) | Yield point (kg/mm <sup>2</sup> ) | Tensile strength (kg/mm <sup>2</sup> ) | Elongation (%)            | Minimum radius capable of 180° bending in transverse direction (Test piece width=200mm) | Hole expanding limit (d/do) (do=20mm) | without pre-strain      |      |
|                                                                              |                           |                           |                                   |                                        |                           |                                                                                         |                                       | after 5% tensile strain |      |
| Steel 1 of the invention                                                     | High temp. finishing type | 6.0                       | 63.8                              | 71.4                                   | 27                        | 0 t                                                                                     | 2.4                                   | 6.8                     | 4.9  |
| Steel 2 "                                                                    |                           | 6.0                       | 65.7                              | 73.5                                   | 27                        | 0 t                                                                                     | 2.8                                   | 7.5                     | 5.6  |
| Steel 3 "                                                                    |                           | 6.0                       | 65.1                              | 72.1                                   | 27                        | 0 t                                                                                     | 2.7                                   | 7.6                     | 5.7  |
| Steel 4 "                                                                    |                           | 10.0                      | 69.2                              | 81.3                                   | 31                        | 0 t                                                                                     | no test                               | 9.8                     | 8.0  |
| Steel 5 "                                                                    |                           | 8.0                       | 62.1                              | 69.3                                   | 28                        | 0 t                                                                                     | 2.9                                   | 12.4                    | 10.1 |
| Steel 6 "                                                                    |                           | 6.0                       | 57.8                              | 68.7                                   | 29                        | 0 t                                                                                     | 2.9                                   | 7.8                     | 5.9  |
| Comparative Steel                                                            |                           | 6.0                       | 52.3                              | 64.5                                   | 30                        | 0.5 t                                                                                   | 1.6                                   | 6.7                     | 4.7  |

Test piece for impact test:

Thickness of product = 6mm: JIS No. 4, Sub-size 5mm

Thickness of product = 8mm and 10mm: JIS No. 4, Sub-size 7.5mm

Table 8

| Rolling conditions and various kinds of characteristic values of Example 4 |             |                            |                                         |                                   |                                        |                              |
|----------------------------------------------------------------------------|-------------|----------------------------|-----------------------------------------|-----------------------------------|----------------------------------------|------------------------------|
| Rolling; Condition                                                         |             |                            |                                         |                                   |                                        |                              |
| Rolling pattern                                                            | Rolling No. | Heating temp. of slab (°C) | Total draft percentage above 1100°C (%) | Each draft % between 1100°C/980°C | Total draft percentage below 980°C (%) | Rolling finishing temp. (°C) |
| A                                                                          | 25          | 1300°C                     | 67%                                     | No rolling                        | 51.5%                                  | 920                          |
|                                                                            | 26          |                            |                                         |                                   |                                        | 880                          |
|                                                                            | 27          |                            |                                         |                                   |                                        | 840                          |
|                                                                            | 30          |                            |                                         |                                   |                                        | 815                          |
|                                                                            | 35          |                            |                                         |                                   |                                        | 780                          |
| B                                                                          | 30          | 1300°C                     | 48%                                     | → 21% → 18% → (Times of pass=2)   | 51.5%                                  | 880                          |
|                                                                            | 31          |                            |                                         | 840                               |                                        |                              |
|                                                                            | 32          |                            |                                         | 810                               |                                        |                              |
|                                                                            | 33          |                            |                                         | 775                               |                                        |                              |
|                                                                            | 34          |                            |                                         | 730                               |                                        |                              |
| J                                                                          | 36          | 1300°C                     | 59%                                     | → 20% → (Times of pass=1)         | 48%                                    | 785                          |

## Notes:

1) Encircles "Rolling number" are belonging to the invention

2) Water-cooling is effected from the end of rolling to 600°C with velocity of 10°C/sec. then furnace cooling from 600°C.

| Mechanical Properties (JIS No. 5) |                                        |                | Cold Workability                                                                         |                                       | Low temperature toughness (JIS No. 4, sub-size 7.5mm) |                         |              |
|-----------------------------------|----------------------------------------|----------------|------------------------------------------------------------------------------------------|---------------------------------------|-------------------------------------------------------|-------------------------|--------------|
| Yield point (Kg/mm <sup>2</sup> ) | Tensile strength (Kg/mm <sup>2</sup> ) | Elongation (%) | Minimum radius capable of 180°C bending in transverse direction (test piece width=200mm) | Hole expanding limit (d/do) (do=20mm) | without pre-strain                                    | after 5% tensile strain | vE-20 (Kg-m) |
| 66.3                              | 74.6                                   | 27.5           | 0.5 t                                                                                    | 2.0                                   | 5.0                                                   | 0.5                     |              |
| 64.1                              | 73.2                                   | 27             | 0.5 t                                                                                    | 2.0                                   | 6.1                                                   | 0.6                     |              |
| 65.0                              | 71.4                                   | 28             | 0 t                                                                                      | 2.2                                   | 7.0                                                   | 1.7                     |              |
| 62.3                              | 69.3                                   | 29             | 0 t                                                                                      | 2.7                                   | 9.8                                                   | 8.1                     |              |
| 60.0                              | 66.8                                   | 29             | 0 t                                                                                      | 2.8                                   | 11.8                                                  | 9.3                     |              |
| 63.0                              | 72.8                                   | 28             | 0.5 t                                                                                    | 2.1                                   | 5.8                                                   | 1.0                     |              |

Rolling conditions and various kinds of characteristic values of Example 4

| Rolling; Condition |      |    |       |     |      |     |
|--------------------|------|----|-------|-----|------|-----|
| 63.1               | 71.0 | 28 | 0 t   | 2.2 | 8.1  | 2.0 |
| 61.5               | 68.6 | 29 | 0 t   | 2.7 | 11.3 | 9.3 |
| 60.8               | 67.9 | 29 | 0 t   | 2.7 | 12.4 | 9.9 |
| 60.7               | 65.5 | 30 | 0 t   | 2.6 | 9.9  | 8.7 |
| 60.3               | 65.0 | 28 | 0.5 t | 2.2 | 8.4  | 4.0 |
| 61.3               | 68.1 | 27 | 0.5 t | 2.2 | 6.9  | 3.4 |

Table 9

| Rolling conditions and various kinds of characteristic values of Example 5 |                                        |                |                                                                                         |                                       |                                                       |                                    |                              |
|----------------------------------------------------------------------------|----------------------------------------|----------------|-----------------------------------------------------------------------------------------|---------------------------------------|-------------------------------------------------------|------------------------------------|------------------------------|
| Rolling Condition                                                          |                                        |                |                                                                                         |                                       |                                                       |                                    |                              |
| Kind of Steel                                                              | Rolling pattern                        | Rolling No.    | Heating temp. of slab (°C)                                                              | Total draft percentage above 1100°C   | Each draft percentage between 1100°C/980°C            | Total draft percentage below 980°C | Rolling finishing temp. (°C) |
| Steel of the invention                                                     | I                                      | 37             | 1270°C                                                                                  | 64%                                   | → 25% →<br>25% →<br>(Times of pass=2)                 | 73%                                | 850                          |
|                                                                            |                                        | 38             |                                                                                         |                                       |                                                       |                                    | 800                          |
| Comparative steel                                                          | I                                      | 22             | 1270°C                                                                                  | 64%                                   | → 25% →<br>25% →<br>(Times of pass=2)                 | 73%                                | 850                          |
|                                                                            | H                                      | 23             | 1270°C                                                                                  | 69%                                   | → 35% →<br>(Times of pass=1)                          | 73%                                | 850                          |
| Mechanical Properties (JIS No. 5)                                          |                                        |                | Cold Workability                                                                        |                                       | Low temperature toughness (JIS No. 4, sub-size 7.5mm) |                                    | Remarks                      |
| Yield point (Kg/mm <sup>2</sup> )                                          | Tensile strength (Kg/mm <sup>2</sup> ) | Elongation (%) | Minimum radius capable of 180° bending in transverse direction (test piece width=200mm) | Hole expanding limit (d/do) (do=20mm) | vE-20 (Kg-m)                                          | without pre-strain                 | after 5% tensile strain      |
| 60.8                                                                       | 69.3                                   | 28             | 0.5 t                                                                                   | 1.9                                   | 5.8                                                   | 1.8                                | Comparative example          |
| 60.5                                                                       | 67.1                                   | 29             | 0 t                                                                                     | 2.7                                   | 10.1                                                  | 8.8                                | The invention                |
| 50.6                                                                       | 63.4                                   | 32             | 0.5 t                                                                                   | 1.9                                   | 9.8                                                   | 7.8                                |                              |
| 51.7                                                                       | 62.7                                   | 33             | 0.5 t                                                                                   | 1.8                                   | 10.6                                                  | 8.5                                |                              |

Notes:

1) Encircles "Rolling No." are belonging to the invention

2) Cooling temperature = 580°C to 620°C

3) Cooling velocity = 7° to 11° C/sec.

Table 10  
Rolling conditions of Example 6

| Rolling pattern          | Heating temp. of slab | Total draft % above 1100°C | Each draft % between 1100°C/980°C  | Total draft % below 980°C | Rolling finishing temp. | Cooling temp. | Cooling velocity |
|--------------------------|-----------------------|----------------------------|------------------------------------|---------------------------|-------------------------|---------------|------------------|
| Low temp. finishing type | 1260°- 1320°C         | more than 50%              | → 20% → 22% →<br>(Times of pass=2) | more than 50%             | 780°-810°C              | 570°- 620°C   | 3-13°C/sec.      |

Table 11

| Various kinds of characteristic values of steel plate obtained by Example 6. |                           |                                   |                                        |                |                                                                                         |                                       |                    |                         |      |                                        |  |
|------------------------------------------------------------------------------|---------------------------|-----------------------------------|----------------------------------------|----------------|-----------------------------------------------------------------------------------------|---------------------------------------|--------------------|-------------------------|------|----------------------------------------|--|
| Manufacturing condition                                                      |                           | Mechanical property (JIS No. 5)   |                                        |                |                                                                                         |                                       |                    | Cold workability        |      | Low temperature toughness vE-20 (kg-m) |  |
| Rolling pattern                                                              | Thickness of product (mm) | Yield point (kg/mm <sup>2</sup> ) | Tensile strength (kg/mm <sup>2</sup> ) | Elongation (%) | Minimum radius capable of 180° bending in transverse direction (test piece width=200mm) | Hole expanding limit (d/do) (do=20mm) | without pre-strain | after 5% tensile strain |      |                                        |  |
| Steel 1 of the invention                                                     | Low temp. finishing type  | 6.0                               | 61.2                                   | 69.4           | 27                                                                                      | 0 t                                   | 2.4                | 6.7                     | 4.7  |                                        |  |
| Steel 2 "                                                                    | "                         | 6.0                               | 62.7                                   | 71.1           | 26                                                                                      | 0 t                                   | 2.7                | 6.8                     | 5.1  |                                        |  |
| Steel 3 "                                                                    | "                         | 6.0                               | 63.1                                   | 71.4           | 27                                                                                      | 0 t                                   | 2.8                | 7.2                     | 5.3  |                                        |  |
| Steel 4 "                                                                    | "                         | 10.0                              | 67.8                                   | 80.6           | 30                                                                                      | 0 t                                   | no test            | 9.7                     | 7.3  |                                        |  |
| Steel 5 "                                                                    | "                         | 8.0                               | 61.2                                   | 68.3           | 28                                                                                      | 0 t                                   | 2.8                | 12.5                    | 10.4 |                                        |  |
| Steel 6 "                                                                    | "                         | 6.0                               | 55.8                                   | 67.1           | 29                                                                                      | 0 t                                   | 2.9                | 7.7                     | 5.7  |                                        |  |
| Comparative Steel 1                                                          | "                         | 6.0                               | 53.1                                   | 64.7           | 29                                                                                      | 0.5 t                                 | 1.6                | 6.6                     | 4.5  |                                        |  |

Note: Test piece for impact test:

Thickness of product = 6mm : JIS No. 4, Sub-size 5mm

Thickness of product = 8mm and 10mm: JIS No. 4, Sub-size 7.5mm

What is claimed is:

1. In a method for manufacturing high tensile steel having superior cold workability and toughness wherein an aluminum killed steel slab is heated and hot rolled, the improvement wherein the steel contains 0.04 to 0.35% Ti, 0.005 to 0.15% soluble aluminum, less than 0.008% N, and Ti/C is less than 4, and the steel slab is heated to greater than 1200°C and the hot rolling is finished at a temperature between 730° and 880°C and carried out with more than one pass at a temperature from 980° to 1100°C and a reduction of more than 28%.

2. In a method for manufacturing high tensile steel having superior cold workability and toughness wherein an aluminum killed steel slab is heated and hot rolled, the improvement wherein the steel contains 0.04 to 0.35% Ti, 0.005 to 0.15% soluble aluminum, less than 0.008% N, And Ti/C is less than 4, and the steel slab is heated to greater than 1200°C and the hot rolling is finished at a temperature between 730° and 815°C and carried out at a temperature below 980°C and a total reduction of more than 50%.

3. The method of claim 2 wherein during the rolling, more than one pass is carried out at a temperature be-

25  
5 between 980° to 1100°C and a reduction of more than 28%

10 4. The method of claim 1 wherein the steel contains 0.03 to 0.20% C, no more than 0.8% Si, 0.90 to 2.5% Mn, no more than 0.020% S, no more than 0.008% N, and the balance iron and unavoidable impurities.

15 5. The method of claim 1, wherein the steel contains one or more of the following: Zr = 0.01 to 0.15%, La + Ce = 0.005 to 0.10%, Nb = 0.01 to 0.10%, V = 0.01 to 0.10%, B  $\leq$  0.0030% Ni  $\leq$  0.5%, Cr  $\leq$  0.5% and Cu  $\leq$  0.5%.

10 6. The method of claim 1 wherein after the hot rolling, the steel is coiled at a temperature in the range from 500° to 680°C.

15 7. The method of claim 6 wherein after the hot rolling and prior to coiling, the steel is cooled at a rate from 3° to 40°C /second.

20 8. The high tensile steel having superior cold workability and toughness produced by the process of claim 1.

25 9. The high tensile steel having superior cold workability and toughness produced by the process of claim 2.

\* \* \* \* \*